

# UNITED STATES PATENT OFFICE.

HUGH CHARLES LOUDON BLOXAM, OF CAPE TOWN, CAPE COLONY, ASSIGNOR  
TO SOUTH AFRICAN MAGANITE EXPLOSIVES SYNDICATE LIMITED, OF  
CAPE TOWN, CAPE COLONY.

## MANUFACTURE OF EXPLOSIVES.

No. 853,056.

Specification of Letters Patent.

Patented May 7, 1907.

Application filed July 12, 1906. Serial No. 325,943.

*To all whom it may concern:*

Be it known that I, HUGH CHARLES LOUDON BLOXAM, a subject of the King of Great Britain, residing at 17 Adderley street, Cape Town, Cape Colony, analytical and consulting chemist, have invented certain new and useful Improvements in the Manufacture of Explosives, of which the following is a specification.

10 Hitherto explosives which have for their principal constituents ammonium nitrate and dinitrobenzene have been made by mixing solid ammonium nitrate with melted dinitrobenzene.

15 By the present invention the ammonium nitrate is melted before it is mixed with the dinitrobenzene or while it is being so mixed, whereby a better explosive is obtained. For instance, one advantage of operating in this manner arises from the fact that the specific 20 gravity of the explosive is much increased, so that the effects of the explosive are more powerful.

The invention is more particularly applicable to the manufacture of an explosive in which ammonium carbonate is added to the mixture of ammonium nitrate and dinitrobenzene, as has been proposed in specification of British Patent No. 7490 of 1904. For 25 instance, ammonium nitrate is heated until it is completely fused and ammonium carbonate is added, or the ammonium carbonate may be added before the fusion. The melt-

ed dinitrobenzene is then run into the fused ammonium nitrate; or the fused ammonium 35 nitrate to which the ammonium carbonate has been added may be run on to the solid dinitrobenzene. In either case the constituents are thoroughly mixed together and after solidification the mixture is ground and 40 made into cartridges, in any known manner. If the dinitrobenzene contains free acid, the latter is neutralized before the mixture is made.

The invention is not limited to any particular proportions, but we have found about 45 83 parts of ammonium nitrate, from 0.5 to 2.5 parts of ammonium carbonate and about 17 parts of dinitrobenzene to be suitable.

Having thus described the nature of my 50 said invention and the best means I know of carrying the same into practical effect, I claim:—

In the process of manufacture of an explosive having for its principal constituents ammonium nitrate and dinitrobenzene, the step 55 which consists in mixing the ammonium nitrate and the dinitrobenzene while they are both in a molten condition.

In witness whereof I have signed my name 60 to this specification in the presence of two subscribing witnesses.

HUGH CHARLES LOUDON BLOXAM.

Witnesses:

WILFRED BRINTON,  
HAROLD BENJAMIN KING TROLLOPE.